

## UNITED STATES PATENT OFFICE.

RENÉ MARIE LOUIS GUSTAVE HÉBERT, OF GISORS, FRANCE, ASSIGNOR TO ALPHONSE VERGÉ, OF PARIS, FRANCE.

PROCESS FOR TREATING COTTON TEXTILES TO IMPART A LINEN-LIKE APPEARANCE THERETO.

No Drawing.

Application filed April 7, 1925. Serial No. 21,445.

To all whom it may concern:

Be it known that I, RENÉ MARIE LOUIS GUSTAVE HÉBERT, a citizen of the Republic of France, residing at Gisors, Eure, France, have invented certain new and useful Improvements in a Process for Treating Cotton Textiles to Impart a Linen-Like Appearance Thereto, of which the following is a specification.

10 This invention relates to a process for treating cotton textiles to impart a linen-like appearance thereto, and essentially consists in scouring the textile material with sodium carbonate ( $Na_2CO_3$ ) and thereafter treating it with dilute sulphuric acid under strictly determined conditions as regards time, temperature and concentration.

It is essential that the fabric be scoured with sodium carbonate ( $Na_2CO_3$ ) under suitable conditions if the desired linen effect is to be fully realized. To this end, the nap or pile of the cotton fabric is completely removed by an effective burning or singeing operation; the material is then ridded of its facing, rinsed and then lixiviated in boiling sodium carbonate ( $Na_2CO_3$ ) in a suitable apparatus and in a continuous operation, whereafter the said fabric is slightly chlorinated and then dried. When the scouring 25 operation is completed, the material is treated with dilute sulphuric acid; this operation may be carried out by means of an ordinary pressing apparatus and a washing machine.

30 The above-mentioned characteristic conditions in which these various operations are to be carried out are as follows:

(1) The strength of the lye must be about 10 grams of sodium carbonate per litre of 35 water.

(2) The degree of concentration of the acid must be between  $53^{\circ}$  and  $53.5^{\circ}$  Bé.

(3) The temperature of the bath must not exceed  $15^{\circ}$  C.

40 (4) The period of impregnation of the fabric with acid must be between 14 and 16 seconds.

The concentration and the period of impregnation may be slightly varied between 45 the said limits in accordance with the nature of the material and is determined for each particular case.

The acid treatment is followed by the dressing operation. The fabric is well rinsed to remove any trace of said acid and is then 55 dried on a tenter-frame to free the threads which the acid treatment has caused to adhere to each other to a greater or lesser extent, more particularly in light textiles, the material being then mercerized according to 60 ordinary practice. After mercerizing, the scouring operation is completed by treating the textile with sodium carbonate ( $Na_2CO_3$ ), chlorine and acid, whereafter it is dried, preferably under simultaneous treatment on 65 the tenter-frame with a little soap and glycerine. The fabric is then moistened, clothed and folded.

Of course, the various stages of the process may be modified to suit particular cases, 70 more particularly as regards dressing, without departing from the spirit of the invention and while still working within the characteristic conditions of acid treatment and scouring with sodium carbonate ( $Na_2CO_3$ ) 75 according to the said invention. Thus for example when treating rather coarse textiles such as cretonne, "longotte" and the like, the thread-freeing stage may be dispensed with, as the threads are much less adhering to each 80 other than in other kinds.

Having now particularly described and ascertained the nature of my said invention and in what manner the same is to be performed, I declare that what I claim is:—

A process for treating cotton textile fabrics to impart the appearance of linen thereto, which comprises scouring the fabric with sodium carbonate, chlorinating the scoured fabric, treating it in a bath of sulphuric acid 90 having a temperature not exceeding  $15^{\circ}$  C. and a concentration between  $53^{\circ}$  and  $53.5^{\circ}$  Bé, the period of impregnation being between 14 and 18 seconds; the two last-mentioned conditions being varied slightly between the said limits in accordance with the nature of the material; rinsing the material after the acid treatment, and thereafter subjecting it to a dressing operation.

In testimony whereof I affix my signature.

RENÉ MARIE LOUIS GUSTAVE HÉBERT.